

No. 820,484.

PATENTED MAY 15, 1906.

H. L. DOHERTY.

## PROCESS OF BURNING CEMENT CLINKER.

APPLICATION FILED DEO. 12, 1905



Witnesses

Henry L. Doherty  
Inventor  
By his attorney  
Sackett & Sack

# UNITED STATES PATENT OFFICE.

HENRY L. DOHERTY, OF MADISON, WISCONSIN.

## PROCESS OF BURNING CEMENT CLINKER.

No. 820,434.

Specification of Letters Patent.

Patented May 15, 1906.

Application filed December 12, 1905. Serial No. 291,460.

*To all whom it may concern:*

Be it known that I, HENRY L. DOHERTY, a citizen of the United States, and a resident of Madison, in the county of Dane and State of Wisconsin, have invented a certain new and useful Process of Burning Cement Clinker, of which the following is a specification.

This invention relates to process of burning Portland cement, which in the best modern practice is burned in rotary inclined or barrel kilns by means of a blast-flame of powdered coal projected from one end of the barrel in heating relation to a continuous stream of the material fed along the floor of the barrel. These instrumentalities I am able to utilize in a new manner and with improved results in respect to the consumption of fuel, the quantity of the product, and the durability of the apparatus. The powdered-fuel blast has hitherto been used with certain objectionable limitations, due particularly to the extremely high temperatures attained and the difficulty of regulating the combustion. Thus, although this method has the advantage of affording a strong flame at a distance from the root of combustion, it is also attended with the disadvantages, among others, of overheating, rapid deterioration of the linings, inflexibility, waste of fuel, and the formation of obstructions in the barrel of the kiln known as "rings," which greatly interfere with the uniform and continuous operation of the kiln.

In burning cement in rotary kilns with the powdered-coal blast it has become customary to employ a non-impinging axial flame, which is preserved from extensive contact with the material and lining by a stratum or envelop of air, an expedient which has the effect of protecting the lining and material to some extent from the intense heat of the flame, but which results in a waste of heat, which I am able to reduce.

My invention, among other things, aims to secure the benefits of the long blast-flame in cement-burning without incurring the aforesaid disadvantages, and particularly does it aim to prevent the formation of the aggregations of unburnt clinker or rings on the walls of the kiln. This I accomplish by using in the air supplied to the kiln for combustion a quantity of diluent gas, the proportion of which I cause to be varied from time to time in order to vary the zone of clinkering from one part of the kiln to another adjacent part. By so doing a better product is obtained and

much fuel saved, since the formation of rings leads to such irregularities of operation that frequently the operation has to be stopped, the kiln cooled, and workmen sent inside to chisel away the obstructing masses. The cause of the formation of rings is due, it appears, to an extended zone of clinkering of such a character that the material is gradually brought from the calcining temperature to the clinkering temperature. By my process the material is subjected to a more sudden change in temperature in passing from the calcining zone to the clinkering zone, and this method of procedure, in conjunction with the variation in the location of the clinkering zone, as will be hereinafter more particularly described, eliminates the tendency to the formation of rings and permits of a uniform uninterrupted operation of the kiln, resulting in a large output and a substantial economy in fuel.

My process consists in passing a continuous stream of cement-forming material through the barrel-kiln, as is customary in the practice of the present day, and in heating the material by a flame produced at the lower end of the kiln through the introduction of powdered fuel in company with a supporter of combustion containing on the average less oxygen than that present normally in air, said oxygen being varied in amount from time to time in order to move the clinkering zone forward or backward in the kiln. This variation in the oxygen content of the supporter of combustion may be periodic—that is, occurring at definite intervals of time—or the variation may be made at irregular intervals, depending upon the condition of the kiln. In order to effect this change in the content of oxygen supplied to the kiln, I prefer, rather than to abstract the oxygen from air, to use a diluent gas—such as, for instance, the waste products of combustion departing as stack-gases.

The carbon dioxide which the stack-gases contain appears to react in some peculiar way with the injected fuel, causing a change in the character of the flame which makes it peculiarly adapted for clinkering and calcining.

I do not lay claim generically to the use of diluent gas as a means for elongating flame, such process being well known in the art.

For the performance of the process herein set forth and claimed I have devised a certain novel combination of apparatus, where-

by the forces and materials concerned in the process are caused to coöperate in the relations necessary for its exercise, which apparatus is also claimed herein.

5 In the accompanying drawing is illustrated a side elevation of a cement-burning furnace equipped to carry out this invention.

In the drawing, 1 is the inclined rotary barrel of a so-called "horizontal" cement-kiln 10 similar to the ordinary although permissibly longer than usual. The barrel has a refractory lining 2, and at its upper end is the stack 3. At this end is also a screw conveyer or feeder 4 for introducing the material. At its 15 lower end is a removable head or hood 5, supporting the blast-nozzle 6 and provided with a stationary outlet 7 for the burnt clinkers. A suitable concentrated fuel, such as powdered coal, is fed to the nozzle 6, in the present case by means of a screw conveyer 8 from a bin or other receptacle into the kiln, with a jet of gaseous fluid delivered through a pipe 9, entering the rear end of the nozzle-pipe or combining-tube.

25 The pipe 9 leads from the chimney 3 and contains a fan-blower 10, which serves to draw back a small portion or modicum of the inert gases or products of substantially complete combustion and force them into the 30 kiln in company with the powdered fuel in predetermined proportion and in company with a predetermined volume of air drawn into the pipe 9 on the suction side of the fan at the point 11, whereat is an adjustable valve 35 or damper for regulating the proportion of air, this damper being conveniently operated by a rod connected to a lever placed near the hood. There is also a damper 12 in the trunk of the pipe for regulating the proportion of 40 stack-gas, although said damper is not commonly changed after having been once set for favorable conditions of operation. The variation in the proportion of oxygen in the blast is accomplished simply by adjusting the 45 valve 11. The wider this damper is opened the greater the amount of air admitted and the smaller is the proportion of stack-gas returned, for the reason that the fan can exhaust only a definite volume at a given 50 speed, and therefore increasing the volume of air means decreasing the volume of stack-gas, and conversely. The kiln-gases contain a percentage of carbon dioxid from the calcination of the lime as well as from combustion.

55 In a well-constructed kiln operating by my process approximately thirty per cent. of carbon dioxid is present in the stack-gases. Combustion may be so conducted as to be substantially complete in the kiln, so that substantially no free oxygen need be present. The proportion of the total kiln-gases returned depends somewhat upon their composition and temperature and also on the quality, temperature, and character of flame desired, &c. If withdrawn from the stack, the

percentage of carbon dioxid will be found much lower than if taken from the mouth of the kiln, owing to the infiltration of air in the space between the kiln and the surrounding wall at its upper end. Frequently the stack-gases withdrawn from the stack itself will contain not over ten per cent. of carbon dioxid. The amount of diluent gas returned may be gaged approximately by the amount of carbon dioxid, for while the carbon dioxid 75 is not the principal diluent, nitrogen being the preponderating gas present, yet as the carbon dioxid bears a fairly constant ratio to the nitrogen the former serves as an index of the dilution. In the mixture entering the 80 kiln I prefer to have not less than one per cent. and not over six per cent. of carbon dioxid or from approximately five per cent. to twenty per cent. of diluent gas. This variation may be secured by the simple adjustment of the damper 11, as above mentioned. The jet of air and coal is introduced into the kiln in such a way that a substantial impingement of the flame against the material occurs. My process makes possible the close contact 90 of the heating agent with the material to be heated, and, as is evident, such a method of heat application results in a pronounced economy in fuel. Frequently the jet may be introduced horizontally and due to the inclination of the kiln and to the height of the material in the kiln an impinging flame is effected without any downward inclination of said jet. It is of course essential that air from extraneous sources be excluded as much 95 as possible. For instance, air entering the lower part of the kiln through the clinker-discharge opening or through the space between the end of the kiln and the hood has a tendency to lift the flame from the material 100 by forming a stratum of cold air in the bottom of the barrel. Such practice, which, in fact, is customary in the present day, I have found to be uneconomical, for besides elevating the flame from the material to a considerable degree, thereby preventing its impingement, the eddies set up from the introduction of said extraneous air cause fluctuations in the flame and lead to irregular operation.

110 While I have disclosed as my preferred embodiment the use of powdered coal as the fuel for producing clinker, I do not limit myself exclusively to such a fuel. The same principles apply in the burning of oil or natural gas and to a considerable degree, moreover, in the combustion of producer-gas.

115 In order to make the variation in the area, locality, and duration of the clinkering zone definitely periodic, I connect the damper 11, by means of a rod or otherwise, to an eccentric working on a shaft driven at a suitable speed, thereby opening and closing the damper at definite intervals. If the material is of such a character that rings form frequently, the periodicity of zone change may be fre- 125 130

quent. Under conditions of operation in which rings are little liable to form I prefer to cause the variations to occur at longer intervals. While it is possible to operate the damper by hand, as shown, yet for simplicity of the operation it is perhaps preferable to render the adjustment automatic, thereby minimizing the duties of the kiln operator.

Element 20 designates a disk revolved by any suitable means (not shown) and carrying a pin 21, adapted to engage a ring 22, carried by rod 23, when the automatic valve operation is desired. When the valve is to be operated by hand, another ring 24 on the rod 23 is to be made to engage a pin 25, carried by lever 26.

What I claim is—

1. Process of burning cement in rotary kilns which consists in conducting combustion of a carbonaceous fuel with air impoverished with respect to its content of oxygen, and in varying the content of oxygen periodically, whereby kiln incrustations are eliminated.

2. Process of burning Portland cement in inclined rotary kilns, said process consisting in burning a stream of carbonaceous fuel in an oxygenated draft; in varying the proportion of oxygen intermittently, and in impinging the resulting flame upon the cementitious material.

3. Process of burning Portland cement in inclined rotary barrels which consists in mixing a stream of powdered fuel with a stream of supporter of combustion under pressure; in varying the composition of said supporter of combustion from time to time, whereby the formation of obstructions in the path of travel of the flame is eliminated, and in bringing the mixture into contact with the cement material at an igniting temperature.

4. Process of burning Portland cement in inclined rotary kilns which consists in passing a stream of cement-forming material continuously through said kiln from its upper to its lower end; in injecting a predetermined amount of powdered coal into said kiln in company with a predetermined amount of air containing products of combustion; in periodically varying proportion of said products of combustion in a predetermined manner; in subjecting the combustible to an igniting temperature; and in bringing the flame produced thereby into intimate contact with said material.

5. Process of burning Portland cement in inclined rotary cement-kilns which consists in introducing a stream of cement-forming ma-

terial into the upper part of said kiln, and in causing same to travel downwardly to the lower end of said kiln; in mingling at the lower end of said kiln a stream of powdered coal with a predetermined amount of air containing products of substantially complete combustion; and periodically varying the composition of said products of combustion whereby the shifting of the clinkering zone is periodically effected; in causing the flame produced by the combustion of said fuel to impinge upon the material; and in preventing the introduction of air from extraneous sources.

6. Process of burning Portland cement in inclined rotary cylindrical kilns; said process consisting in subjecting the cement material to an impinging flame produced by injecting a mixture of powdered coal and diluted air as a single jet against said material; and in periodically varying the degree of dilution of said diluted air.

7. Process of burning Portland cement in inclined rotary cylindrical kilns which consists in conducting the combustion of carbonaceous fuel with a supporter of combustion; and in periodically varying the composition of said supporter of combustion.

8. Process of burning Portland cement which consists in burning carbonaceous fuel in contact with the cement material with a supporter of combustion containing carbon dioxide; and in intermittently varying the proportion of said carbon dioxide whereby kiln incrustations are minimized.

9. Process of burning Portland cement in inclined rotary cylindrical barrels, said process consisting in exposing a flattened stream of cement-forming material to the calcining and clinkering action of a blast of powdered coal, said coal being introduced as a single jet with sufficient oxygen to complete combustion, and with other gases of an inert character; in subjecting the fuel mixture to an igniting temperature whereby a flame of high temperature is developed; in causing said flame to impinge upon said flattened stream of cement material; in periodically varying the proportion of inert gases introduced with said coal; and in preventing the admission of air from extraneous sources.

Signed at New York, in the county of New York and State of New York, this 5th day of December, A. D. 1905.

HENRY L. DOHERTY.

Witnesses:

FLETCHER P. SCOFIELD,  
J. CHAS. ANDREWS.